

C. E. ARNOLD.

METHOD OF FORMING ARTIFICIAL LEATHER AND THE PRODUCT THEREOF.

APPLICATION FILED OCT. 23, 1915.

1,350,271.

Patented Aug. 17, 1920.

Fig. 1



Fig. 2



INVENTOR  
Charles Elwood Arnold  
BY -  
Brinsford Wright & Smale  
ATTORNEYS

# UNITED STATES PATENT OFFICE.

CHARLES ELWOOD ARNOLD, OF WILMINGTON, DELAWARE, ASSIGNOR TO DU PONT  
FABRIKOID COMPANY, OF WILMINGTON, DELAWARE, A CORPORATION OF  
DELAWARE.

## METHOD OF FORMING ARTIFICIAL LEATHER AND THE PRODUCT THEREOF.

1,350,271.

Specification of Letters Patent. Patented Aug. 17, 1920.

Application filed October 23, 1915. Serial No. 57,416.

To all whom it may concern:

Be it known that I, CHARLES ELWOOD ARNOLD, of Wilmington, in the county of New Castle and in the State of Delaware, have invented a certain new and useful Improvement in Methods of Forming Artificial Leather and the Product Thereof, and do hereby declare that the following is a full, clear, and exact description thereof.

10 My invention relates to a process of producing coated fabrics whereby an artificial leather of great efficiency and high quality is produced, and the product thereof. Hitherto it has been customary in producing artificial leather to apply a layer of coating material upon the surface of a fabric, usually a woven fabric, which fabric was so constructed that the layer of coating material merely adhered to the surface thereof.

15 This was due to the fact that the fibers of the fabric used were located close together. The product thus previously produced comprised a body of fabric having adhering to the surface thereof a layer of the coating material. Artificial leather thus constructed was comprised of a comparatively weak outer surface and a comparatively strong under surface, the weaker portion being the layer of coating material and the stronger portion being the fabric to the surface of which it adheres. Furthermore there was a more or less weak bond of union between the layer of coating material and the body of fabric.

20 The object of my invention is to provide a process for producing artificial leather and the product thereof, in which the artificial leather has its layer or layers of coating material strengthened by a light open mesh fabric embedded in the coating material, the light open mesh fabric serving the purpose primarily of strengthening the layer of coating material so as to thus provide a strengthened layer of coating material which approximates closely in strength and length of wear the backing which is applied thereto. A further object of my invention is to provide an open mesh fabric which is especially adapted for the production of the type of artificial leather above referred to.

25 Further objects of my invention will appear from the detailed description herein-after.

While my invention is capable of embodiment in many different forms, for the purpose of illustration I have shown only one form thereof in the accompanying drawings in which,

30 Figure 1 is a plan view of an open mesh fabric adapted to be used in producing artificial leather in accordance with my invention; and

35 Fig. 2 is a section of a piece of artificial leather made in accordance with my invention.

40 In the drawings I have shown a body of open mesh fabric 1 having openings 2. The fabric which I may use for this purpose may be any one of many different kinds, and may be of silk, cotton, wool or any other fiber, but I have found it especially advantageous to use the light fabric known as cotton leno weave, or a leno weave in which the filler is silk and the warp cotton. This fabric is especially advantageous for the production of the artificial leather made in accordance with my invention as the openings 2 therein are maintained securely and in a uniform manner, owing to a twist 3 that is given to certain of the threads throughout the fabric. The characteristic of this type of fabric is furthermore the fact that it is very resistant to being pulled out of shape. In other words, it is resistant to the sliding of the warp threads along the filler threads. Preferably the fabric is one having about forty (40) threads to the inch. This fabric is preferably first immersed in a solution of nitrocellulose dissolved in a suitable solvent and in which the proportions are

45 preferably 2 ounces of nitro cellulose to a gallon of solvent, the solvent being preferably comprised of benzol 60 parts, and ethyl acetate 40 parts. This composition is in the form of a thin solution, and after being applied to the fabric is dried thereon so as to leave on the fabric a thin coating 1<sup>a</sup> which reduces the diagonal stretch of the fabric to a minimum. This does not result in filling the openings 2, but stiffens and strengthens the threads thereof. To such a body of open mesh fabric I apply a layer of a plastic coating material, which may be a pyroxylin composition, a composition containing drying oils, or a rubber composition. In the case where a pyroxylin com-

55

60

65

70

75

80

85

90

95

100

105

position is used, said composition may be comprised of the following constituents in the proportions given:

|   |               |           |
|---|---------------|-----------|
| 5 | Pyroxylin     | 120 parts |
|   | Camphor       | 30 parts  |
|   | Castor oil    | 250 parts |
|   | Benzol        | 60 parts  |
|   | Ethyl acetate | 40 parts  |

10 Instead, however, the plastic composition used may contain celluloid scrap and castor oil as in the following composition:

|    |                 |           |
|----|-----------------|-----------|
| 15 | Celluloid scrap | 150 parts |
|    | Castor oil      | 250 parts |
|    | Benzol          | 60 parts  |
|    | Ethyl acetate   | 40 parts  |

A layer of the plastic composition 4 is then applied to the open mesh fabric 1 by rolling the composition into the same, as for example, with calender rolls. If desired a similar layer 5 of the plastic composition is applied to the other surface of the open mesh fabric 1. Thereafter, if desired, one or more

25 additional coatings may be applied to either or both sides of the product, thus produced. For these additional coatings, however, I preferably apply layers 6 and 7 of a composition in the form of a jelly. This composition also may be of any one of the above types of coating composition, but preferably I make use of a pyroxylin jelly which may be comprised of the following constituents in the proportions given:

|    |                 |     |
|----|-----------------|-----|
| 35 | Nitro cellulose | 10% |
|    | Benzol          | 40% |
|    | Ethyl acetate   | 28% |
|    | Castor oil      | 17% |
| 40 | Pigment         | 5%  |

45 It will be understood that any number of such coatings as those named hereinabove may be applied to either one or both surfaces of the body of the fabric 1.

50 The film thus produced and having the open mesh fabric 1 embedded therein, is of great strength and shows a wearing test two or three times higher than any grade of artificial leather previously obtainable. In order to give thickness and increased strength to the film thus produced, the latter is combined with or cemented to a suitable backing 8 which may be sheeting, drill, sateen or felt, the cement used being of any desired kind, but which may be composed of the following constituents in the proportions given:

55 32 ozs. nitrocellulose and 4 ozs. camphor in one gallon of solvent consisting of 60 parts by volume of benzol and 40 parts ethyl acetate.

60 In my invention it is not absolutely necessary to immerse the fabric in the thin solution of pyroxylin, but it has been found that 65 solutions of other materials may be used for

the same purpose, or that this step may be omitted altogether if desired. It is furthermore not essential to apply the plastic by rolling, as it may be applied in any other suitable way. It is also to be understood 70 that no particular composition is essential to my invention, nor is it to be confined necessarily to any particular fabric.

While I have described my invention above in detail, I wish it to be understood 75 that many changes may be made therein without departing from the spirit of my invention.

I claim:

1. The process which comprises embedding 80 a light fabric in a coating composition, the fabric having previously had its diagonal stretch reduced by the application of a coating.

2. The process which comprises embedding 85 a leno weave fabric in a coating composition, the fabric having previously had its diagonal stretch reduced by the application of a coating.

3. The process which comprises embedding 90 a light textile fabric in a coating composition, and then combining the same with a fabric backing.

4. The process which comprises embedding 95 a leno weave fabric in a coating composition, and then combining the same with a fabric backing.

5. The process which comprises embedding 100 a light fabric in a coating composition, the fabric having previously had its diagonal stretch reduced by the application of a coating, and then combining the same with a fabric backing.

6. The process which comprises embedding 105 a leno weave fabric in a coating composition, the fabric having previously had its diagonal stretch reduced by the application of a coating, and then combining the same with a fabric backing.

7. The process which comprises embedding 110 a light fabric in a pyroxylin coating composition, the fabric having previously had its diagonal stretch reduced by the application of a coating.

8. The process which comprises embedding 115 a leno weave fabric in a pyroxylin coating composition, the fabric having previously had its diagonal stretch reduced by the application of a coating.

9. The process which comprises embedding 120 a light fabric in a pyroxylin coating composition, and then combining the same with a fabric backing.

10. The process which comprises embedding 125 a leno weave fabric in a pyroxylin coating composition, and then combining the same with a fabric backing.

11. The process which comprises embedding 130 a light fabric in a pyroxylin coating composition, the fabric having previously

- had its diagonal stretch reduced by the application of a coating, and then combining the same with a fabric backing.
12. The process which comprises embedding a leno weave fabric in a pyroxylin coating composition, the fabric having previously had its diagonal stretch reduced by the application of a coating, and then combining the same with a fabric backing.
- 10 13. The process which comprises embedding a light fabric in a pyroxylin coating composition, the fabric having previously had its diagonal stretch reduced by the application of a coating, said composition being in the form of a plastic, then applying one or more pyroxylin jelly coats, and then combining the same with a fabric backing.
- 15 14. The process which comprises embedding a leno weave fabric in a pyroxylin coating composition, the fabric having previously had its diagonal stretch reduced by the application of a coating, said composition being in the form of a plastic, then applying one or more pyroxylin jelly coats, and then combining the same with a fabric backing.
- 20 15. An artificial leather comprising a leno weave fabric embedded in a coating composition.
- 30 16. An artificial leather comprising a light fabric embedded in a coating composition, the fabric having first had its diagonal stretch reduced before being so embedded.
- 35 17. An artificial leather comprising a leno weave fabric embedded in a coating composition, the fabric having first had its diagonal stretch reduced before being so embedded.
- 40 18. The process which consists in immersing an open mesh fabric in a thin nitrocellulose solution and then filling the interstices of the fabric with a plastic composition.
- 45 19. The process which consists in immersing an open mesh fabric in a thin nitrocellulose solution and then filling the interstices of the fabric with a pyroxylin plastic composition.
- 50 20. The process which consists in immersing an open mesh fabric in a solution having a volatile thin solvent, drying the fabric, and filling the interstices thereof with a plastic composition.
- 55 21. The process which consists in immersing an open mesh fabric in a solution having a volatile thin solvent, drying the fabric, and filling the interstices thereof with a pyroxylin plastic composition.
- 60 22. An artificial leather comprising a light textile fabric embedded in a coating composition, and a fabric backing combined therewith.
23. An artificial leather comprising a leno weave fabric embedded in a coating composition, and a fabric backing combined therewith.
24. An artificial leather comprising a light fabric embedded in a coating composition, the fabric having first had its diagonal stretch reduced before being so embedded, and, a fabric backing combined therewith.
25. An artificial leather comprising a leno weave fabric embedded in a coating composition, the fabric having first had its diagonal stretch reduced before being so embedded, and a fabric backing combined therewith.
- 30 26. An artificial leather comprising a leno weave fabric embedded in a pyroxylin coating composition.
- 35 27. An artificial leather comprising a light fabric embedded in a pyroxylin coating composition, the fabric having first had its diagonal stretch reduced before being so embedded.
- 40 28. An artificial leather comprising a leno weave fabric embedded in a pyroxylin coating composition, the fabric having first had its diagonal stretch reduced before being so embedded.
- 45 29. An artificial leather comprising a light fabric embedded in a pyroxylin coating composition, and a fabric backing combined therewith.
- 50 30. An artificial leather comprising a leno weave fabric embedded in a pyroxylin coating composition, and a fabric backing combined therewith.
- 55 31. An artificial leather comprising a light fabric embedded in a pyroxylin coating composition, the fabric having first had its diagonal stretch reduced before being so embedded, and a fabric backing combined therewith.
- 60 32. An artificial leather comprising a leno weave fabric embedded in a pyroxylin coating composition, the fabric having first had its diagonal stretch reduced before being so embedded, and a fabric backing combined therewith.
- 65 33. The process which comprises embedding a light weight open mesh fabric in a coating composition, the fabric having previously had its diagonal stretch reduced by the application of a coating.
- 70 34. An artificial leather comprising a backing, a coating of pyroxylin composition thereon, and a light weight fabric embedded in said coating and reinforcing the same.
- 75 35. An artificial leather comprising a backing, a coating of pyroxylin composition thereon, and a light weight fabric embedded in said coating and reinforcing the same, the coating on the two sides of said fabric being united through the interstices thereof.

- 2E
36. An artificial leather comprising a backing, a coating of pyroxylin composition thereon, and a light weight fabric embedded in said coating and reinforcing the same, 5 the coating on the two sides of said fabric being united through the interstices thereof, said fabric having had its diagonal stretch reduced previous to being embedded in said composition.
- 10 37. An artificial leather comprising a fabric backing, a coating composition thereon, and a light weight fabric embedded in said coating and reinforcing the same, the

coating on the two sides of said fabric being united through the interstices thereof. 15

38. An artificial leather comprising a fabric backing, a coating of pyroxylin composition thereon, and a light weight fabric embedded in said coating and reinforcing the same. 20

In testimony that I claim the foregoing I have hereunto set my hand.

CHARLES ELWOOD ARNOLD.

Witnesses:

P. E. STRICKLAND,  
HARRY J. HAWKE.